# EUROPEAN PATENT SPECIFICATION

(11) **EP 2 963 142 B1**
(45) Date of publication and mention of the grant of the patent: **24.02.2021**
(21) Application number: 15174636.9
(22) Date of filing: 30.06.2015
(51) Int. Cl.: C23C 4/10, C23C 4/12, C23C 4/11, C23C 4/134

(54) **SYSTEMS AND METHODS FOR PLASMA SPRAY COATING**
SYSTEME UND VERFAHREN ZUR PLASMASPRÜHBESCHICHTUNG
SYSTÈMES ET PROCÉDÉS DE REVÊTEMENT PAR PULVÉRISATION DE PLASMA

(30) Priority: 30.06.2014 US 201462019012 P
(43) Date of publication of application: 06.01.2016
(73) Proprietor: United Technologies Corporation, Farmington, CT 06032 (US)
(72) Inventor: THAYER, Henry H., Wethersfield, CT 06109 (US); RIZZO, John P., Vernon, CT 06066 (US)
(74) Representative: Dehns

(56) References cited:
- EP-A2- 0 246 596
- WO-A1-2006/074549
- WO-A1-2013/126134
- US-A- 4 076 883
- US-A1- 2003 068 518
- US-A1- 2014 154 422

## Description

### FIELD

The present disclosure relates to systems and methods for applying coatings, and more particularly, to systems and methods for filament plasma spray coating.

### BACKGROUND

Plasma spraying of fine powders can be very challenging in terms of the size of coating material that may be employed and the carrying medium utilized. For example, gas fed particles and liquid suspensions may result in clumping and/or uneven application of the powder. Further, a liquid suspension such as a water suspension can cool a plasma jet while a flammable liquid can create handling issues. Thus, there is a need in the art for improved plasma spraying systems and methods which utilize powders.

US 2003/0068518, WO 2006/074549 and EP 0246596 are all concerned with techniques for applying coatings.

### BRIEF SUMMARY OF THE EMBODIMENTS

Disclosed and claimed herein are systems and methods for plasma spraying. The present invention provides a method for plasma spraying according to claim 1 and a plasma spraying system according to claim 5.

In one embodiment, the filament is an elongated material formed with a diameter in the range of 0.1 mm to 1 mm.

In one embodiment, powder particles embedded within the filament have a diameter in the range of 1 nm to 0.001 cm.

In one embodiment, controlling application of filament includes applying the filament to the plasma jet at a controlled rate.

In one embodiment, the filament is fed axially or radially into the plasma jet.

In one embodiment, the method for plasma spraying further includes controlling a plasma source to generate a plasma jet.

In one embodiment, the embedded powder particles are plasticized by the plasma jet to form a coating for the substrate.

In one embodiment, the method for plasma spraying further includes controlling the position of at least one of a substrate and plasma device during coating or spraying.

Other aspects, features, and techniques will be apparent to one skilled in the relevant art in view of the following detailed description of the embodiments.

### BRIEF DESCRIPTION OF THE DRAWINGS

The features, objects, and advantages of the present disclosure will become more apparent from the detailed description set forth below when taken in conjunction with the drawings in which like reference characters identify correspondingly throughout and wherein:
FIG. 1 depicts an exemplary process for plasma spraying according to one or more embodiments;
FIG. 2 depicts a graphical representation of a plasma spraying system according to one or more embodiments;
FIG. 3 depicts a graphical representation of an axial feed plasma spraying system according to one or more embodiments; and
FIG. 4 depicts a graphical representation of an axial feed plasma spraying system according to one or more embodiments.

### DETAILED DESCRIPTION OF THE EXEMPLARY EMBODIMENTS

### Overview and Terminology

One aspect of this disclosure relates to plasma spraying components. In one embodiment, a method for plasma spraying includes application of a filament embedded with one or more powders, such as a fine ceramic powder, to a plasma jet to generate plasticized ceramic particles which impact a substrate, freeze, and form a ceramic coating. In another embodiment, a system is provided including a feed element for the filament and at least a controller to control application of the filament to a plasma jet.

In one embodiment, fine, or very fine (e.g., nano fine) ceramic powder is embedded in an organic filament during a filament extrusion process. The filament is then fed into a plasma jet at a controlled rate, similar to a wire spray process. Once exposed to the plasma jet, the organic filament burns away and the ceramic powder is plasticized and accelerated by the plasma jet, and flies through the air to the substrate where it deposits as a ceramic coating.

As used herein, the terms "a" or "an" shall mean one or more than one. The term "plurality" shall mean two or more than two. The term "another" is defined as a second or more. The terms "including" and/or "having" are open ended (e.g., comprising). The term "or" as used herein is to be interpreted as inclusive or meaning any one or any combination. Therefore, "A, B or C" means "any of the following: A; B; C; A and B; A and C; B and C; A, B and C". An exception to this definition will occur only when a combination of elements, functions, steps or acts are in some way inherently mutually exclusive.

Reference throughout this document to "one embodiment," "certain embodiments," "an embodiment," or similar term means that a particular feature, structure, or characteristic described in connection with the embodiment is included in at least one embodiment. Thus, the appearances of such phrases in various places throughout this specification are not necessarily all referring to the same embodiment. Furthermore, the particular features, structures, or characteristics may be combined in any suitable manner on one or more embodiments without limitation.

### Exemplary Embodiments

Referring now to the figures, FIG. 1 depicts process **100** for plasma spraying according to one or more embodiments. Process **100** may be initiated at block **105** with controlling a plasma source, such as the plasma source of FIGs. 2-4, to generate a plasma jet configured to burn away filament material and generate a plasticized spray for coating a substrate with the plasticized ceramic of the spray.

At block **110,** process **100** controls feed of a filament embedded with powder to a plasma jet at a controlled rate to generate a plasma spray for coating a substrate. As further discussed below, the filament may be fed axially or radially into the plasma jet. The plasma spray generated by the plasma jet and filament forms a wear or heat resistant coating on the substrate. The rate of feed of the filament to a plasma device can vary in accordance with the type of device utilized. The feed rate may depend on, for example, the amount of oxygen and fuel fed into a High Velocity Oxy-Fuel device. Similarly, the filament feed rate can be adjusted based on the power level in the plasma gun.

Process **100** may optionally include controlling the position of the substrate and/or plasma source in some embodiments. At block **115,** positioning of the substrate and/or the plasma source may also be controlled.

FIG. 2 depicts a graphical representation of a plasma spraying system according to one or more embodiments. System **200** includes a feed device **205,** a plasma device **220,** and a controller **245** configured to control or operate the feed device **205** to output a filament **210** to a plasma device **220.** The plasma device **220** produces a plasma jet **225** which receives the filament **210** and generates coating spray **230.** The coating spray **230** can include one or more plasticized ceramic particles or powder, and forms a coating **235** on substrate **240.**

Feed device **205** is configured to store and output filament **210.** In certain embodiments, feed device **205** includes a rotational spool **206** controlled by controller **245** to output filament **210** at a controlled rate. In certain embodiments, feed wheels **211** and **212** are configured to guide and/or draw filament from feed device **205.**

Filament **210** is an organic binder material including ceramic powder particles embedded in the organic material. Filament **210** may be formed as an elongated material (e.g., string, rod, tube, etc.) with a diameter in the range of 0.1 mm to 1 mm. Similarly, powder particles **215** embedded within the filament **210,** which may be ceramic particles, can have a diameter in the range of 1 nm to 0.001 cm. As filament **210** is applied to the plasma jet **225** at a controlled rate, the plasma jet **225** burns the organic filament away, plasticizes the ceramic powder embedded in the filament, and accelerates the plasticized ceramic to substrate **240** where it deposits as a ceramic coating **235.** Filament **210** is embedded with a fine powder and into an organic filament, like nylon, polyester, polyurethane, etc.

Filament **210** may be very thin, on the order of 1 mm or less and may use a fairly high concentration of ceramic, such as Aluminum Oxide (Alumina) or Yttrium Oxide (Yttiria). The bend radius of filament **210** may depend on the filament diameter and ceramic concentration. Bend radius can affect how filaments are stored. In accordance with the present disclosure, fine, or nano fine, ceramic powder is embedded in an organic filament **210.** In one embodiment, the powder particles **215** may be embedded by feeding the powder into the molten plastic during an extrusion process.

In certain embodiments, filament **210** may be formed with one or more shapes (e.g., with its cross-section or outer surface having a particular shape) to allow for one or more shapes or pellets to be generated by system **200.** Utilizing a filament **210** with a particular cross-sectional or shape in system **200** allows for different coverage for the coating **235** to the substrate **240** during plasma spraying due to differences in plasticizing due to the particular shapes. Similarly, applying a particular cross-sectional shape to filament **210** provides different coverage during plasma spraying due to differences in velocity of the plasticized ceramic due to shape. Exemplary cross-sectional shapes of filament **210** include, but are not limited to, circular, square, rectangular, triangular, star, oval, etc.

Controller **245** may be configured to control the position of at least one of the substrate **240** and plasma source **220** during coating or spraying. Plasma source **220** may be configured to output plasma jet **225** based on one or more control signals received from controller **245.** Plasma source **220** may be an electric-arc source, high velocity oxy-fuel (HVOF) source, and/or thermal source in general.

Coating spray **230** includes plasticized ceramic **231.** The melted ceramic **231** is formed from the particles **215** of filament **210.** The ceramic may be one of aluminum oxide or other ceramic powders, including, but not limited to Yttria Stabilized Zirconia, Aluminum Oxide (Alumina) or Yttrium Oxide (Yttiria). By providing an extruded filament **210,** nano fine ceramic powder can be fed to a plasma jet to allow for even application without clumping of the powder particles. Similarly, nano fine powders can be used without generating the handling issues of conventional liquid suspension techniques. In addition, providing an extruded filament **210** with nano fine ceramic powder to plasma jet **225** produces a ceramic coating with a columnar structure. Columnar structures provide greater shear resistance. In addition, the waste stream is easier to handle than the waste stream from conventional spray techniques, such as liquid feed spray techniques.

According to one embodiment, plasma jet **225** burns off the organic material of the filament such that the plasticized particles can create coating **235** on substrate **240.**

System **200** depicts a radial arrangement for feeding filament **210** to a plasma jet. It will be appreciated that the principles of operation of system **200** are similar to the arrangements described below with respect to FIGs. 3-4.

FIG. 3 depicts a graphical representation of an axial feed plasma spraying system **300** according to one or more embodiments. System **300** includes feed device **205,** and plasma device **320,** the feed device **205** configured to output filament **210** to plasma device **320.**

System **300** is an axial feed configuration, and feeds filament **210** through an axial cavity, such as a channel **321,** of plasma device **320.** System **300** includes guide rollers **311** configured to receive the filament **210** from feed device **205.** Feed rollers **312** feed filament **210** into plasma device **320.** Plasma device **320** includes the channel **321** to receive and guide the filament **210.** The diameter or width of the channel **321** is slightly larger than the filament **210** to be received. Filament **210** may be fed to plasma device **320** with inert gas such that the inert gas aids to advance the filament **210** through the receiving channel **321** and prevents melted filament from sticking within the channel **321** of the plasma device **320.**

According to one embodiment, the plasma device **320** is an electric arc type plasma device for generating a plasma jet **325.** Cathode(s) **345,** anode(s) **350** and power supply **355** are configured to generate electric arcs to generate plasma jet **325** using inert gas, usually argon, which is blown through the arc to excite the gas.

Filament **210** is fed into plasma device **320** and is melted by plasma jet **325.** The melted powder, shown as **322,** is formed from ceramic particles **215** of filament **210** that are entrained in plasma jet **325** to form coating spray **330.** Coating spray **330** forms a coating **235** on substrate **240.** In one embodiment, organic binder material of the filament **210** is burned away by plasma source **325** such that spray **330** includes only, or substantially only, ceramic material (e.g., non-binder material) of the filament. System **300** may include a controller (e.g., controller **245**) which may be employed to control operation of plasma device **320** and/or feed device **205.**

FIG. 4 depicts a graphical representation of an axial feed plasma spraying system **400** according to one or more embodiments. System **400** includes a feed device **205,** and a plasma device **420.** The feed device **205** is configured to output a filament **210** to the plasma device 420.

System **400** is an axial feed configuration configured to feed the filament **210** through an axial cavity of plasma device **420.** System **400** includes guide roller **411** configured to receive filament **210** from feed device **205.** Feed rollers **412** feed filament **210** into plasma device **420.** Plasma device **420** may include a channel to receive the filament, the channel having an opening or diameter slightly larger than the filament **210.** Filament **210** may be fed to plasma device **420** with inert gas such that the inert gas aids to advance the filament **210** through the receiving channel and prevents sticking of the filament in the plasma device **420.**

According to one embodiment, plasma device **420** is a High Velocity Oxy-Feed (HVOF) plasma device for generating a plasma jet **425.** The plasma device **420** is configured to receive oxygen **441** and fuel (e.g., propane, propylene, or hydrogen, etc.) **442** via channels **445** and **450,** respectively. Plasma device **420** is configured to supply oxygen to burn away binder material of filament **210.** The configuration of plasma device **420** allows for filament **210** to be exposed to and inserted in the plasma jet **425.** Oxygen **441** and fuel **442** are mixed and ignited in plasma device **420** to generate plasma jet **425.** Fuel **442** is used for burning away the binder and plasticizing the powder particles of filament **210.** Filament **210** is fed into plasma device **420** and melted by plasma jet **425** such that ceramic particles in filament **210** are entrained in plasma jet **425** to form coating spray **430.** In one embodiment, organic binder material of the filament **210** is burned away by plasma source **425** such that spray **430** includes only, or substantially, ceramic material (e.g., non-binder material) of the filament.

Coating spray **430** forms a coating **235** on substrate **240.** System **400** may include a controller (e.g., controller **245**) which may be employed to control operation of plasma device **420** and/or feed device **205.**

While this disclosure has been particularly shown and described with references to exemplary embodiments thereof, it will be understood by those skilled in the art that various changes in form and details may be made therein without departing from the scope of the claims.

## Claims

1. A method for plasma spraying, the method comprising controlling application of a filament (210) wherein the filament (210) is formed of an organic binder material and is embedded with ceramic powder particles (215) to a plasma jet (225;325;425) to burn the organic binder material and to plasticize the ceramic powder particles (215) to generate a spray (230;330;430) that includes the plasticized ceramic coating (235) for coating a substrate (240).

2. The method for plasma spraying of claim 1, further comprising controlling a plasma source to generate a plasma jet (225;325;425).

3. The method for plasma spraying according to claim 2, wherein the embedded powder particles (215) are plasticized by the plasma jet (225;325;425) to form a coating for the substrate (240).

4. The method for plasma spraying of claim 1, 2 or 3 further comprising controlling the position of at least one of a substrate (240) and plasma device (220;320;420) during coating or spraying.

5. A plasma spraying system (200;300;400) comprising:
a plasma source (206);
a filament feed element (205) configured to store and output a filament (210) wherein the filament (210) is formed of an organic binder material and is embedded with ceramic powder particles (215); and
a controller (245) coupled to the plasma source (206) and filament feed element (205), wherein the controller (245) is configured to:
control a plasma source (206) to generate a plasma jet (225;325;425); and
control application of the filament (210) to the plasma jet (225;325;425) to burn the organic binder material and to plasticize the ceramic powder particles (215) to generate a spray (230;330;430) that includes the plasticized ceramic coating (235) for coating a substrate (240).

6. The method or system of any preceding claim, wherein the filament (210) is an elongated material formed with a diameter in the range of 0.1 mm to 1 mm.

7. The method or system of any preceding claim, wherein powder particles (215) embedded within the filament have a diameter in the range of 1 nm to 0.001 cm.

8. The method or system of any preceding claim, wherein controlling application of the filament (210) includes application of the filament (210) to the plasma jet (225;325;425) at a controlled rate.

9. The method or system of any preceding claim, wherein the filament (210) is fed axially or radially into the plasma jet (225;325;425).

10. The system of any of claims 5 to 9, the controller (245) further configured to control a position of at least one of a substrate (240) and plasma device (220) during coating or spraying.

11. The system of any of claims 5 to 10, wherein the feed element (205) includes one or more of a spool element (206) and filament storage area.

12. The system of any of claims 5 to 11, wherein the system includes one or more rollers (211;212;311;312;411;412) to apply the filament (210) to the plasma jet (225;325;425).

## Patentansprüche

1. Verfahren zum Plasmasprühen, wobei das Verfahren ein Steuern des Auftragens eines Filaments (210), wobei das Filament (210) aus einem organischen Bindemittel ausgebildet ist und keramische Pulverpartikel (215) darin eingebettet sind, auf einen Plasmastrahl (225; 325; 425) umfasst, um das organische Bindemittel zu verbrennen und die keramischen Pulverpartikel (215) zu plastifizieren, um einen Sprühnebel (230; 330; 430), der die plastifizierte Keramikbeschichtung (235) beinhaltet, für die Beschichtung eines Substrats (240) zu erzeugen.

2. Verfahren zum Plasmasprühen nach Anspruch 1, ferner umfassend ein Steuern einer Plasmaquelle derart, dass sie einen Plasmastrahl (225; 325; 425) erzeugt.

3. Verfahren zum Plasmasprühen nach Anspruch 2, wobei die eingebetteten Pulverpartikel (215) durch den Plasmastrahl (225; 325; 425) plastifiziert werden, um eine Beschichtung für das Substrat (240) zu bilden.

4. Verfahren zum Plasmasprühen nach Anspruch 1, 2 oder 3, ferner umfassend ein Steuern der Position mindestens eines von einem Substrat (240) und einer Plasmavorrichtung (220; 320; 420) während des Beschichtens oder Sprühens.

5. Plasmasprühsystem (200; 300; 400), umfassend:
eine Plasmaquelle (206);
ein Filament-Einspeiseelement (205), das dazu konfiguriert ist, ein Filament (210) zu lagern und auszugeben, wobei das Filament (210) aus einem organischen Bindemittel ausgebildet ist und keramische Pulverpartikel (215) darin eingebettet sind; und
eine Steuerung (245), die an die Plasmaquelle (206) und das Filament-Einspeiseelement (205) gekoppelt ist, wobei die Steuerung (245) für Folgendes konfiguriert ist:
Steuern einer Plasmaquelle (206) derart, dass sie einen Plasmastrahl (225; 325; 425) erzeugt; und
Steuern des Auftragens des Filaments (210) auf den Plasmastrahl (225; 325; 425), um das organische Bindemittel zu verbrennen und die keramischen Pulverpartikel (215) zu plastifizieren, um einen Sprühnebel (230; 330; 430), der die plastifizierte Keramikbeschichtung (235) beinhaltet, für die Beschichtung eines Substrats (240) zu erzeugen.

6. Verfahren oder System nach einem der vorhergehenden Ansprüche, wobei es sich bei dem Filament (210) um ein längliches Material handelt, das mit einem Durchmesser im Bereich von 0,1 mm bis 1 mm ausgebildet ist.

7. Verfahren oder System nach einem der vorhergehenden Ansprüche, wobei die in das Filament eingebetteten Pulverpartikel (215) einen Durchmesser im Bereich von 1 nm bis 0,001 cm aufweisen.

8. Verfahren oder System nach einem der vorhergehenden Ansprüche, wobei das Steuern des Auftragens des Filaments (210) ein Auftragen des Filaments (210) auf den Plasmastrahl (225; 325; 425) mit einer gesteuerten Rate beinhaltet.

9. Verfahren oder System nach einem der vorhergehenden Ansprüche, wobei das Filament (210) axial oder radial in den Plasmastrahl (225; 325; 425) eingespeist wird.

10. System nach einem der Ansprüche 5 bis 9, wobei die Steuerung (245) ferner dazu konfiguriert ist, eine Position mindestens eines von einem Substrat (240) und einer Plasmavorrichtung (220) während des Beschichtens oder Sprühens zu steuern.

11. System nach einem der Ansprüche 5 bis 10, wobei das Einspeiseelement (205) eines oder mehrere von einem Spulenelement (206) und einem Filament-Lagerbereich beinhaltet.

12. System nach einem der Ansprüche 5 bis 11, wobei das System eine oder mehrere Walzen (211; 212; 311; 312; 411; 412) zum Auftragen des Filaments (210) auf den Plasmastrahl (225; 325; 425) beinhaltet.

## Revendications

1. Procédé de pulvérisation de plasma, le procédé comprenant la commande de l'application d'un filament (210) dans lequel le filament (210) est formé d'un matériau liant organique et est incorporé avec des particules de poudre céramique (215) à un jet de plasma (225 ; 325 ; 425) pour brûler le matériau liant organique et pour plastifier les particules de poudre céramique (215) afin de générer un spray (230 ; 330 ; 430) qui comporte le revêtement céramique plastifié (235) pour revêtir un substrat (240).

2. Procédé de pulvérisation de plasma selon la revendication 1, comprenant en outre la commande d'une source de plasma pour générer un jet de plasma (225 ; 325 ; 425).

3. Procédé de pulvérisation de plasma selon la revendication 2, dans lequel les particules de poudre incorporées (215) sont plastifiées par le jet de plasma (225 ; 325 ; 425) pour former un revêtement pour le substrat (240).

4. Procédé de pulvérisation de plasma selon la revendication 1, 2 ou 3, comprenant en outre la commande de la position d'au moins l'un parmi un substrat (240) et un dispositif à plasma (220 ; 320 ; 420) pendant le revêtement ou la pulvérisation.

5. Système de pulvérisation de plasma (200 ; 300 ; 400) comprenant :
une source de plasma (206) ;
un élément d'alimentation en filament (205) configuré pour stocker et produire un filament (210) dans lequel le filament (210) est formé d'un matériau liant organique et est incorporé avec des particules de poudre céramique (215) ; et
un dispositif de commande (245), couplé à la source de plasma (206) et à l'élément d'alimentation en filament (205), dans lequel le dispositif de commande (245) est configuré pour :
commander une source de plasma (206) pour générer un jet de plasma (225 ; 325 ; 425) ; et
commander l'application du filament (210) au jet de plasma (225 ; 325 ; 425) pour brûler le matériau liant organique et plastifier les particules de poudre céramique (215) afin de générer un spray (230 ; 330 ; 430) qui comporte le revêtement céramique plastifié (235) pour revêtir un substrat (240).

6. Procédé ou système selon une quelconque revendication précédente, dans lequel le filament (210) est un matériau allongé formé avec un diamètre dans la plage de 0,1 mm à 1 mm.

7. Procédé ou système selon une quelconque revendication précédente, dans lequel les particules de poudre (215) incorporées à l'intérieur du filament ont un diamètre dans la plage de 1 nm à 0,001 cm.

8. Procédé ou système selon une quelconque revendication précédente, dans lequel la commande de l'application du filament (210) comporte l'application du filament (210) au jet de plasma (225 ; 325 ; 425) à une vitesse commandée.

9. Procédé ou système selon une quelconque revendication précédente, dans lequel le filament (210) est alimenté axialement ou radialement dans le jet de plasma (225 ; 325 ; 425) .

10. Système selon l'une quelconque des revendications 5 à 9, le dispositif de commande (245) étant en outre configuré pour commander une position d'au moins l'un parmi un substrat (240) et un dispositif à plasma (220) pendant le revêtement ou la pulvérisation.

11. Système selon l'une quelconque des revendications 5 à 10, dans lequel l'élément d'alimentation (205) comporte un ou plusieurs parmi un élément de bobine (206) et une zone de stockage de filament.

12. Système selon l'une quelconque des revendications 5 à 11, dans lequel le système comporte un ou plusieurs rouleaux (211 ; 212 ; 311 ; 312 ; 411 ; 412) pour appliquer le filament (210) au jet de plasma (225 ; 325 ; 425).
